

## UNITED STATES PATENT OFFICE

HAROLD R. RAFTON, OF LAWRENCE, MASSACHUSETTS, ASSIGNOR TO RAFFOLD PROCESS CORPORATION, A CORPORATION OF MASSACHUSETTS

## METHOD OF PRODUCING PAPER FILLED WITH ALKALINE FILLER

No Drawing. Application filed November 24, 1928. Serial No. 321,753.

This invention relates to the manufacture of paper and more particularly to a method of producing paper filled with alkaline filler.

The principal object of my invention is to provide a method for the reduction, elimination, prevention or alteration of foam in the manufacture of a substantially unsized paper filled with alkaline filler.

An important object of my invention is to improve machine operation in such manufacture, particularly as regards the dandy roll.

Another object of my invention is to avoid the deterioration by alkaline filler of the effect of alum in a paper mix.

15 A further object of my invention is to avoid the deterioration in a substantially unsized paper filled with alkaline filler of a precipitate of alum and an amount of rosin size insufficient to impart a substantial degree of 20 sizing to the paper.

25 A further object of my invention is to avoid the deterioration in a substantially unsized paper filled with alkaline filler of a precipitate formed from a soluble salt such as sodium silicate and a precipitant such as alum.

30 A further object of my invention is to provide a process of making substantially unsized paper filled with alkaline filler wherein 35 in alkaline filler is added to the paper mix at such a point in the process that the time and intimacy of contact of the alkaline filler in the paper mix are materially limited.

40 A further object of my invention is to provide a process of making substantially unsized paper filled with alkaline filler wherein the alkaline filler is added at the wet end of the paper machine.

45 Other objects and advantages of my invention will become apparent during the course of the following description.

In my copending application Serial No. 304,167 filed September 5, 1928, I have disclosed and claimed a method whereby sized paper filled with alkaline filler may be made by adding alkaline filler to the previously sized paper stock at the wet end of the paper machine. The present application deals with the manufacture by a similar method of sub-

stantially unsized paper filled with alkaline filler.

As set forth in my copending applications Serial Nos. 304,171 and 304,174, both filed September 5, 1928, I have found that in the manufacture of substantially unsized papers filled with alkaline filler it is highly desirable in order to improve the running of the paper on the machine and in order to improve the quality of paper made to add alum at the wet end of the paper machine, or to add rosin size in the beater, precipitate it with alum, and thereafter restore the effectiveness of the precipitate by a further addition of alum at the wet end of the paper machine, or to add rosin size in the beater followed by the addition of alum at the wet end of the paper machine, in either of the two latter cases the size used being in an amount insufficient to impart a substantial degree of sizing to the paper.

Likewise in my copending applications Serial Nos. 319,719 and 319,720 both filed November 15, 1928, I disclose and claim a method of incorporating soluble material such as sodium silicate into paper, either by the addition of sodium silicate in the beater where it is precipitated as by alum, and the effectiveness of the resulting precipitate restored as by a further quantity of alum added at the wet end of the paper machine, or by the addition of sodium silicate in the beater followed by the addition of alum at the wet end of the paper machine.

In the latter mentioned four copending applications the presence of alkaline filler in the relatively concentrated fibrous mix is recognized as being the cause of the necessity of adding alum at the wet end of the paper machine in order to achieve the various results desired, and it is by this step that the desired effects are capable of accomplishment. I have discovered, however, that these effects can be equally well attained by adding the alum, or rosin size, in an amount insufficient to impart a substantial degree of sizing to the paper, and alum, or sodium silicate and alum, to the relatively concentrated fibrous mix as in the beater, and then adding the alkaline filler at the wet end of the paper ma-

chine. By this method in the one case a substantially foam free paper and good machine operating conditions can be obtained; and in the other the beneficial effect of sodium silicate-alum precipitate in the stock and paper made therefrom can be retained.

I have found that the damaging or destructive effect of the alkaline filler to the above referred desired effects is a function of the time of contact of the alkaline filler with the constituents of the mix and also of its intimacy of contact with these constituents. I have also discovered that the intimacy of contact of the alkaline filler with the constituents of the mix resulting from high concentrations and/or agitation is particularly damaging to these effects. I have further found that if the time of contact be greatly reduced over that which normally would obtain in the ordinary papermaking process, and the conditions made such that intimacy of contact is also greatly reduced, the tendency for the alkaline filler to injure or destroy these effects is greatly reduced, if not entirely eliminated.

The method which I employ consists substantially in adding an alkaline filler at a point in the papermaking process where the intimacy of contact and the time of contact of the alkaline filler and the constituents of the mix will be at a minimum. In accordance with my invention, I may add the alkaline filler at a point where the mix is still in a relatively concentrated condition provided that the time of contact in such condition is to be relatively short, but the preferred procedure is to add the alkaline filler at or subsequent to the point where the mix is diluted preparatory to its delivery to the web-forming device, i. e., at the wet end of the paper machine. From this point to the point of web formation the time of contact is short and the intimacy of contact is practically at a minimum owing to the high dilution.

Inasmuch as the white water from a paper machine running on a stock containing alkaline filler contains a considerable quantity of this filler, it is preferable not to use such white water either in the beater, the beater chest, at the Jordan, or in the machine chest, as in any of these places the constituents of the mix in a relatively concentrated condition will come into contact with the alkaline filler for a relatively long period of time, and this will tend to injure or destroy the effects desired. The exception to this case is where the white water to be employed has been clarified or filtered so that there is a negligible quantity of the alkaline filter present in such purified water, and in this case such water may be used in the places which are stated above to be places at which it is preferable not to use the unpurified white water.

In the preferred practice of my invention I add to the beater or other similar machine,

all the fibrous materials to be used, with the exception of those fibrous materials coming under the definition of alkaline filler herein-after set forth and such fibrous material as is present in the stock recovered from the white water. I also add to the beater alum, or rosin size, in an amount insufficient to impart a substantial degree of sizing to the paper, or sodium silicate and alum, or both rosin size and sodium silicate and alum. In any event I prefer to have an excess of alum present. Filler other than alkaline filler may be added if desired, as well as coloring matter or the like.

After the usual treatment in the beater, the mix is preferably passed through the beater chest, Jordan, and machine chest in the customary manner. This procedure and/or order of steps is not essential, and may vary considerably as will be apparent to one skilled in the art. The mix, still in relatively concentrated form, is now at the point where it is ready for dilution preparatory to delivery to the web-forming end of the paper machine. As indicated above, all water used for dilution up to this point in the process is preferably either fresh water, or white water which has been purified so that it contains only a negligible amount of alkaline filler. However, at this point, untreated white water as obtained from the paper machine may be used as diluting water. During dilution at this point, or subsequent thereto, the alkaline filler preferably in aqueous suspension is added continuously, due care being taken that adequate mixing is insured.

According to the definition of alkaline filler hereinafter set forth, this term includes fibrous matter in combination with the mineral alkaline filler itself. In such cases the fibrous material must be properly broken down in a suitable apparatus before addition as will be apparent. It may be refined separately if desired, but ordinarily this will be unnecessary as such fibres have already been refined in the previous papermaking procedure.

Moreover, the stock recovered from the white water contains alkaline filler and this stock preferably should not be added at a point prior to the point of dilution preparatory to delivery to the web-forming end of the paper machine as the content of alkaline filler would tend to injure or destroy the effects desired because of the relatively prolonged contact in a relatively concentrated condition.

Moreover, the recovery of the stock from the white water should take place as soon as possible after the production of the white water and such stock should preferably be returned promptly to its point of reuse so as to afford as little time as possible for contact between the alkaline filler and the constitu-

ents of the mix which have accompanied it in the white water.

If the recovered stock be obtained from a settling system, a convenient way is to add the recovered stock directly from this settling system continuously at the mixing box at the point of dilution of the stock. If the stock is recovered by a filter or deckering system by mixing the white water with relatively concentrated stock as a "sweetener", then a convenient method is to divert part or all of the stream of concentrated fibrous stock just before its delivery to the mixing box, and utilize this as "sweetener" stock, delivering it after it has so functioned to the mixing box. In this way the stock containing the alkaline filler derived from the white water remains for only a brief interval in concentrated condition, and is quickly diluted at the mixing box.

Of course it is also possible to use the procedure of adding alkaline filler at the wet end of the paper machine to a paper mix in which no alum or other material adversely affected by alkaline filler is present. In such case of course this method of adding alkaline filler would be chiefly of value in increasing the beater capacity in regard to fibrous constituents, and also in permitting beating to be accomplished more effectively, as the mechanically protecting action of the fibre by the filler would be avoided.

Instead of rosin size, which may be referred to as sodium resinate, and which may therefore be termed an alkali metal salt, any other size is suitable which is used in conjunction with a size precipitant as alum. One example of such a size is a soap, such as an oleate. Another is a wholly or partially saponified wax, such as beeswax.

Instead of alum, for example as a precipitant for the rosin size, I may use acidic material such as sulphuric acid, or sodium bisulphate ( $NaHSO_4$ ), or other salts of aluminum, but from the standpoints of efficiency and cost I prefer alum. In the case of the use of alum as a precipitant for sodium silicate, I may also substitute in addition to the above, ammonium salts such as the chloride or the sulphate.

It is thus apparent that other acidic material as sulphuric acid, or other metallic salts as sodium bisulphate, or salts of aluminum other than alum, or in certain cases ammonium salts are equivalents of alum in the practice of my invention.

Instead of sodium silicate, I may use sodium stannate, or any of the other inorganic alkali metal salts with a pH value greater than 7.0, which are precipitable by material which depresses their hydroxyl ion concentration.

An illustrative furnish suitable for practicing my invention is:

*Materials added in beater*

|                                                                                                    | Pounds  |
|----------------------------------------------------------------------------------------------------|---------|
| Fibrous furnish (air dry basis), e. g. equal parts of sulphite pulp, soda pulp and old paper stock | 1700 70 |
| Alum                                                                                               | 40      |

*Material added proportionately and continuously on dilution*

|                                                                               | Pounds |
|-------------------------------------------------------------------------------|--------|
| Alkaline filler (bone dry basis), e. g. calcium carbonate magnesium hydroxide | 75 300 |
|                                                                               |        |

Another illustrative furnish is:

*Material added in beater*

|                                                                                                    | Pounds |
|----------------------------------------------------------------------------------------------------|--------|
| Fibrous furnish (air dry basis), e. g. equal parts of sulphite pulp, soda pulp and old paper stock | 1700   |
| Rosin size                                                                                         | 6      |
| Alum                                                                                               | 50     |

*Material added proportionately and continuously on dilution*

|                                                                               | Pounds |
|-------------------------------------------------------------------------------|--------|
| Alkaline filler (bone dry basis), e. g. calcium carbonate magnesium hydroxide | 90 300 |
|                                                                               |        |

Another illustrative furnish is:

*Material added in beater*

|                                                                                | Pounds |
|--------------------------------------------------------------------------------|--------|
| Fibrous material (air dry basis), e. g. equal parts of sulphite and soda pulps | 1700   |
| Inorganic alkali metal salt, e. g. 60° Bé. sodium silicate                     | 30 100 |
| Precipitant, e. g. alum                                                        | 45     |

*Material added proportionately and continuously on dilution*

|                                                                               | Pounds |
|-------------------------------------------------------------------------------|--------|
| Alkaline filler (bone dry basis), e. g. calcium carbonate magnesium hydroxide | 90 300 |
|                                                                               |        |

Another illustrative furnish is:

*Material added in beater*

|                                                                                | Pounds |
|--------------------------------------------------------------------------------|--------|
| Fibrous material (air dry basis), e. g. equal parts of sulphite and soda pulps | 1700   |
| Rosin size                                                                     | 6 115  |
| Inorganic alkali metal salt, e. g. 60° Bé. sodium silicate                     | 30     |

|      | Pounds |
|------|--------|
| Alum | 60     |
|      |        |

*Material added proportionately and continuously on dilution*

|                                                                               | Pounds  |
|-------------------------------------------------------------------------------|---------|
| Alkaline filler (bone dry basis), e. g. calcium carbonate magnesium hydroxide | 300 125 |
|                                                                               |         |

It is to be understood that the above furnishes are illustrative only and not limiting, as I have found that my invention may be practiced with a wide variety of ingredients in the furnish, with widely varying proportions.

tions of the several ingredients to one another, for making a wide variety of grades of paper.

- As will be apparent from the previous detailed description it is very desirable to be able to utilize in a paper mix both an acidic constituent, such as alum or a small amount of precipitated sodium resinate accompanied usually by excess alum, and a substantially water insoluble alkaline constituent, such as an alkaline filler. These two constituents, however, under conditions obtaining in the ordinary method of paper manufacture, react chemically upon one another so that the effect of the acidic constituent is deteriorated if not completely destroyed. The primary object of this invention is to so adjust conditions as to substantially prevent the acidic constituent from reacting chemically with the alkaline filler and thus to preserve the desired effect of the acidic constituent in the paper-making mix. This result is attained as indicated above by adjusting conditions so that the alkaline filler is brought into contact with the paper mix containing the acidic constituent under circumstances which tend to prevent the chemical reaction between the alkaline filler and the acidic constituent, that is, under conditions favoring the minimizing of the time and intimacy of contact of the constituents of the mix, or specifically, at the wet end of the paper machine. It is thus obvious that conditions are adjusted to prevent rather than to obtain a chemical reaction between the acidic constituent and the alkaline filler.
- A chemical reaction between acidic material and alkaline material which is to result in a final state which is substantially in the vicinity of neutrality obviously requires the employment of substantially chemically equivalent proportions of the two materials. Thus if it were desired to effect such a reaction between the acidic constituent, e. g. alum, and alkaline filler, substantially chemical equivalents of each would have to be employed. A stoichiometrical calculation shows that if for example calcium carbonate were to be the alkaline filler used, one part thereof would be chemically equivalent to 2.2 parts of commercial alum. If calcium carbonate magnesium hydroxide (of equimolecular proportions) were to be the alkaline filler used, one part thereof would be chemically equivalent to 2.9 parts of alum.
- In the present invention, however, no such chemically equivalent proportions of calcium carbonate and alum are used, but rather the amount of alkaline filler used is far in excess of the chemical equivalent of the alum used. This is made clear by reference to the illustrative furnishes given above. In these furnishes 40 to 60 lbs. of alum and 300 lbs. of alkaline filler, in this instance calcium carbonate magnesium hydroxide, are employed. In some of the formulas, a considerable por-

tion of the alum is used up in precipitating size and/or sodium silicate; hence for the purpose of this calculation it can be assumed that in the illustrative furnishes there would be present approximately 40 to 50 lbs. of "free", i. e. uncombined alum. Using the figure of 50 lbs. alum, this would give therefore a ratio of alkaline filler, in this case calcium carbonate magnesium hydroxide, to uncombined or "free" alum of 17.4 to 2.9. Thus it is apparent that in this case there is present 17.4 times the amount of alkaline filler which would be the chemical equivalent of the alum, that is, 17.4 times the amount of alkaline filler necessary to react completely with the alum were conditions provided favorable for the consummation of reaction between the two.

It is thus apparent that I use an amount of alkaline filler far in excess of the chemical equivalent of alum employed. Thus even were conditions such that the alkaline filler were acted upon by the alum, as is substantially not the case in my invention, under such conditions the unacted upon residual alkaline filler would only be slightly less in amount than that originally added and thus substantially the same amount as added (less, of course, the losses through the machine wire into the white water) would find its way into the paper. While I have not limited my invention to the addition of any definite amount of alkaline filler in relation to the total furnish, the examples of illustrative furnishes given indicate that the proportion of alkaline filler normally present constitutes a substantial percentage of the total furnish, and thus the paper produced by my process would contain a substantial percentage of alkaline filler and would be what is known in the art as "paper filled with alkaline filler".

On the other hand if instead of using alkaline filler as is my practice in an amount far in excess of the alum used, alkaline filler were employed only in an amount chemically equivalent to the "free" alum present, it can be readily seen from the following computation that such an amount of alkaline filler would not produce a paper which would be considered as a "paper filled with alkaline filler". In order to compute the amount of alkaline filler that would be chemically equivalent in amount to the alum, it is only necessary to know how much alum is ordinarily used. Whereas I have not limited my invention to the addition of any definite amount of alum in relation to the total furnish, it is apparent from the examples of illustrative furnishes above, that the proportion of "free" alum used on the total furnish normally runs in the vicinity of several percent. If, for example, I use 2½% of free alum on the total furnish, which is approximately the amount given in the illustrative

furnishes above, the amount of alkaline filler chemically equivalent thereto would be, in the case of calcium carbonate, 1.1%, and in the case of calcium carbonate magnesium hydroxide .9% on the total furnish. The resulting paper would of course contain smaller percentages of filler owing to losses of filler through the machine wire into the white waters. Such amounts of filler therefore or even amounts to some excess thereof (such as would be present if the alkaline filler were used in amounts chemically equivalent to quantities of alum somewhat larger than that given above) would be wholly inadequate to impart any substantial degree of filling to the paper made with such furnish. Indeed in such case analytical procedures of fairly exact degree of refinement would have to be employed to detect the presence of such minute quantity of alkaline filler that might find its way into the paper to distinguish it with certainty for instance from the small amounts of inorganic constituents naturally occurring in the fibres, such as sulphite or soda fibres. On the other hand the filler in paper ordinarily known as "filled" paper, such as that to which my invention is directed, is present in so much larger amount that the normal inorganic constituents of the fibre are negligible in proportion thereto, and ordinary ashing of the paper by ignition gives a result indicating the filler content sufficiently accurately for practical paper mill purposes.

It is thus clearly evident that I add alkaline filler at the wet end of the paper machine to prevent the chemical reaction between the alkaline filler and the acidic constituent of the mix, and therefore my invention is completely differentiated from any papermaking procedure wherein alkaline filler would be added to a paper mix in proportion substantially chemically equivalent to the acidic constituent thereof, for chemically reacting purposes.

It is to be noted that in any papermaking procedure where it would have been desired to add alkali for chemically reacting purposes at the dilute stage, for example for neutralizing the acidic content of a paper mix, a proportion of alkali chemically equivalent to that of the acidic content would have been employed. This chemical equivalence would according to the prior knowledge of the art have been a necessary and limiting feature of such procedure. Were soluble alkali in excess of the chemical equivalent of the acid added, the mix would have been alkalinized. No distinction would have been made according to prior knowledge between soluble and substantially insoluble alkali. According to known prior art, were substantially insoluble alkali used as a substitute for the soluble alkali, it would have been subject to the same limitations as to quantity em-

ployed, and were there used an amount of insoluble alkali, for example alkaline filler, in excess of that chemically equivalent to the acidic content of the mix, the prior art would have taught that there would also have resulted an alkalinizing of the mix, thereby defeating the neutralizing purpose for which the alkali would have been added. It was not until the discovery herein disclosed that it was realized that an amount of alkaline filler greatly in excess of the chemical equivalent of the acidic constituent could be added at the dilute stage without thereby destroying or substantially deteriorating the effect of the acidic constituent in the mix. Hence the present invention distinctly differentiates from any chemically reacting, i. e. neutralizing practice, as the addition of alkali at the dilute stage in such practice would necessarily have been confined by previously existing knowledge to the addition of proportions chemically equivalent to the acidic constituent of the mix.

It is also clear that my invention is directed to the manufacture of paper filled in substantial degree with alkaline filler, and is thus completely differentiated from any papermaking procedure in which alkaline filler would be added in proportion substantially chemically equivalent to the acidic constituent, as in the latter case a commercially wholly inconsequential amount of alkaline filler, if indeed any quantity at all detectable by ordinary analytical procedure, would be incorporated into the paper, and such paper could not be considered in the ordinary papermaking interpretation of the words as "paper filled with alkaline filler".

When I use the expression "alkali metal", I mean to include the hypothetical alkali metal ammonium ( $\text{NH}_4$ ).

By the term "alkaline filler" I mean filler which when agitated in contact with freshly boiled distilled water, say for an hour, will impart a pH value to such water greater than 7.0, that is, which will be on the alkaline side of the neutral point. Among fillers included in this group may be mentioned calcium carbonate, of which lime mud from the causticizing process is one form; calcium carbonate magnesium basic carbonate employed in the paper disclosed in my U. S. Patent No. 1,595,416, issued August 10, 1926; calcium carbonate magnesium hydroxide disclosed in my U. S. Patent No. 1,415,391, issued May 9, 1922; and other substantially water insoluble normal or basic carbonates of alkaline earth metals (which expression is herein intended to include magnesium), or compounds, double salts, or physically associated mixtures of these with one or more other acid soluble materials of a substantially water insoluble nature.

By the term "alkaline filler" I also intend to include fibrous material and/or other ma-

terial such as paper coating constituents or the like containing one or more compounds of the character referred to, such as "old papers" or similar papers, "broke", or the like.

5 When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

15 By the term "wet end of the paper machine" I intend to include those instrumentalities employed in paper manufacture by which and/or in which a relatively concentrated paper mix is diluted, and treated, conveyed or fed up to the point of web-formation such as the mixing box, regulating and proportioning devices, rifflers, troughs, screens, head boxes, inlets, and the like, including also instrumentalities used in the white water cycle.

20 25 While I have described in detail the preferred embodiment of my invention, it is to be understood that the details of procedure, the proportions of ingredients, and the arrangement of steps may be widely varied 30 without departing from the spirit of my invention or the scope of the subjoined claims.

I claim:

1. That step in the method of manufacturing a substantially unsized paper filled with 35 alkaline filler comprising adding alkaline filler, in an amount sufficient to impart a substantial degree of filling to the resulting paper, to fibrous material under conditions favoring the minimizing of the time of contact of the alkaline filler and the fibrous material.

40 2. That step in the method of manufacturing a substantially unsized paper filled with alkaline filler comprising adding alkaline filler, in an amount sufficient to impart a substantial degree of filling to the resulting paper, to fibrous material under conditions favoring the minimizing of the time and intimacy of contact of the alkaline filler and the fibrous material.

45 50 3. The method of manufacturing a substantially unsized paper filled with alkaline filler comprising adding to fibrous material previously mixed with alum alkaline filler, in an amount sufficient to impart a substantial degree of filling to the resulting paper, under conditions favoring the minimizing of the time of contact of the alkaline filler and the fibrous mix, and thereafter making paper therefrom.

55 60 4. The method of manufacturing a substantially unsized paper filled with alkaline filler comprising adding to fibrous material previously mixed with alum alkaline filler, in an amount sufficient to impart a substantial degree of filling to the resulting paper,

under conditions favoring the minimizing of the intimacy and time of contact of the alkaline filler and the fibrous mix, and thereafter making paper therefrom.

5 70 5. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with acidic material, and thereafter making paper therefrom.

75 6. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with a salt of aluminum, and thereafter making paper therefrom.

80 7. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with alum, and thereafter making paper therefrom.

85 8. The method of manufacturing a substantially unsized paper filled with alkaline filler comprising adding alkaline filler, in an amount sufficient to impart a substantial degree of filling to the resulting paper, at the wet end of the paper machine to a paper stock which has been previously mixed with a precipitant for an ingredient of said stock.

90 9. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with soluble material and a precipitant therefor, and thereafter making paper therefrom.

95 10. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with alkali metal salt and a precipitant therefor, and thereafter making paper therefrom.

11. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with alkali metal salt comprising size, in an amount insufficient to produce a substantial degree of sizing, and

120

130

135

140

145

150

155

160

165

170

175

180

185

190

1. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with sodium silicate and rosin size, in an amount insufficient to produce a substantial degree of sizing, and a precipitant therefor, and thereafter making paper therefrom. 70
2. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with alkali metal salt comprising rosin size, in an amount insufficient to produce a substantial degree of sizing, and a precipitant therefor, and thereafter making paper therefrom. 75
3. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with an inorganic alkali metal salt with a pH value greater than 7.0, which is precipitable by material which depresses its hydroxyl ion concentration, and alkali metal salt comprising size, 80 in an amount insufficient to produce a substantial degree of sizing, and precipitant for said alkali metal salts, and thereafter making paper therefrom. 85
4. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with an inorganic alkali metal salt with a pH value greater than 7.0, which is precipitable by material which depresses its hydroxyl ion concentration, and alkali metal salt comprising rosin size, in an amount insufficient to produce a substantial degree of sizing, and precipitant for said alkali metal salts, and thereafter making paper therefrom. 90
5. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with sodium silicate and rosin size, in an amount insufficient to produce a substantial degree of sizing, and alum, and thereafter making paper therefrom. 95
6. That step in the manufacture of substantially unsized paper filled with alkaline filler comprising the addition of alkaline filler to fibrous material at the wet end of the paper machine in an amount sufficient to impart a substantial degree of filling to the resulting paper. 100
7. That step in the manufacture of substantially unsized paper filled with alkaline filler comprising the addition of alkaline filler consisting of alkaline earth metal compound to fibrous material at the wet end of the paper machine in an amount sufficient to impart a substantial degree of filling to the resulting paper. 105
8. That step in the manufacture of substantially unsized paper filled with alkaline filler comprising the addition of alkaline filler consisting of calcium carbonate to fibrous material at the wet end of the paper machine in an amount sufficient to impart a substantial degree of filling to the resulting paper. 110
9. That step in the manufacture of substantially unsized paper filled with alkaline filler comprising the addition of alkaline filler consisting of calcium carbonate and magnesium compound to fibrous material at the wet end of the paper machine in an amount sufficient to impart a substantial degree of filling to the resulting paper. 115
10. That step in the manufacture of substantially unsized paper filled with alkaline filler comprising adding alkaline filler, in an amount sufficient to impart a substantial degree of filling to the resulting paper, at the wet end of the paper machine to fibrous material previously mixed with sodium silicate and rosin size, in an amount insufficient to produce a substantial degree of sizing, and precipitant for said sodium silicate and said size, and thereafter making paper therefrom. 120
11. The method of manufacturing a substantially unsized paper filled with alkaline filler comprising adding alkaline filler, in an amount sufficient to impart a substantial degree of filling to the resulting paper, at the wet end of the paper machine to fibrous material previously mixed with sodium silicate and rosin size, in an amount insufficient to produce a substantial degree of sizing, and precipitant for said sodium silicate and said size, and thereafter making paper therefrom. 125

filler comprising the addition of alkaline filler consisting of calcium carbonate magnesium hydroxide to fibrous material at the wet end of the paper machine in an amount sufficient to impart a substantial degree of filling to the resulting paper.

25. The cyclic procedure in the method of making substantially unsized paper filled with alkaline filler, comprising the addition of alkaline filler to fibrous material at the wet end of the paper machine in an amount sufficient to impart a substantial degree of filling to the resulting paper, and the returning of the material recovered from the white water 10 to the wet end of the paper machine.

26. The method of producing substantially unsized paper filled with alkaline filler comprising adding alkaline filler, in an amount sufficient to impart a substantial degree of filling to the resulting paper, to the paper mix 20 at a point not in advance of that at which the concentrated stock is ready for dilution.

27. The method of producing a substantially unsized paper filled with alkaline filler, 25 comprising adding alkaline filler, in an amount sufficient to impart a substantial degree of filling to the resulting paper, at the wet end of the paper machine to a fibrous mix to which a metallic salt has been previously 30 added, and thereafter making paper therefrom.

28. The method of producing a substantially unsized paper filled with alkaline filler, comprising adding alkaline filler consisting 35 of alkaline earth metal compound, in an amount sufficient to impart a substantial degree of filling to the resulting paper, at the wet end of the paper machine to a fibrous mix to which a metallic salt has been previously 40 added, and thereafter making paper therefrom.

29. The method of producing a substantially unsized paper filled with alkaline filler, comprising adding alkaline filler consisting 45 of calcium carbonate, in an amount sufficient to impart a substantial degree of filling to the resulting paper, at the wet end of the paper machine to a fibrous mix to which a metallic salt has been previously added, and thereafter 50 making paper therefrom.

30. The method of producing a substantially unsized paper filled with alkaline filler, comprising adding alkaline filler consisting 55 of calcium carbonate and magnesium compound, in an amount sufficient to impart a substantial degree of filling to the resulting paper, at the wet end of the paper machine to a fibrous mix to which a metallic salt has been previously added, and thereafter 60 making paper therefrom.

31. The method of producing a substantially unsized paper filled with alkaline filler, comprising adding alkaline filler consisting 65 of calcium carbonate magnesium hydroxide, in an amount sufficient to impart a substan-

tial degree of filling to the resulting paper, at the wet end of the paper machine to a fibrous mix to which a metallic salt has been previously added, and thereafter making paper therefrom.

In testimony whereof I affix my signature.

HAROLD ROBERT RAFTON.

70

75

80

85

90

95

100

105

110

115

120

125

130